

## UNITED STATES PATENT OFFICE.

MALCOLM SPARKES, OF LONDON, ENGLAND.

## PROCESS FOR COLORING THE SURFACE OF WOOD.

No Drawing.

Application filed November 21, 1925. Serial No. 70,691.

The invention relates particularly to the coloring of the surface of wood by chemical action instead of by liquid stain. On all woods with a strongly pronounced hard and soft grain the use of liquid stains produces an unsatisfactory and negative result, due to the soft portion of the timber absorbing most of the color while the hard grain is scarcely affected.

10 The invention has in view overcoming this difficulty by giving a balanced coloring to both the hard and soft grain, thereby preserving and enhancing the natural color values. A further object of the invention is 15 so as to color inexpensive timbers that they may be raised to the front rank of decorative materials.

To these ends the invention primarily consists in treating the surface of the wood with 20 a metallic sulphate and a developing reagent, and if desired with ammonia. The invention includes woods treated by the new process.

The developing reagents may either be such as develop the color owing to the action 25 of metal-containing salts, or be such as develop the color owing to a bleaching action. Among the former reagents may be mentioned the chromates, in particular, the bi-chromates and among the latter oxalic acid.

30 The purpose of the developing reagent is to intensify or correct the effect produced by the effect of the metallic sulphate.

The metallic sulphate and developing reagent are employed in solution and the choice 35 of the particular sulphate and whether the sulphate and the reagent are employed simultaneously or successively depend upon the particular wood and the effect it is desired to obtain. The resultant tones may be modified or improved by the addition of the ammonia which may be either in liquid or gaseous form.

40 Three examples of carrying out the process are given below, but the invention is not limited to these examples:

*Example 1 Oregon pine.*

The surface of the wood is treated with a 45 solution of ferrous sulphate (2 oz. to the gallon) applied evenly with a sponge. It is then allowed to stand until the moisture has evaporated. It is then re-treated with a solution of potassium bichromate (2 oz. to the gallon) to which has been added 4 ounces of 50 .880 liquid ammonia, and the moisture again evaporated. The result is a cool dark brown

color, which can be finished by wax polish, French polish or varnish.

*Example 2 western hemlock.*

60 The surface of the wood is treated with a solution of ferrous sulphate (2 oz. to the gallon) applied as before. As soon as the moisture has evaporated it is then re-treated with a solution of oxalic acid (2 oz. to the gallon) 65 followed after evaporation by a wash of liquid ammonia diluted in the proportion of one of ammonia to four of water. The result is a delicate silver grey which darkens slightly on exposure to strong sunlight, and 70 may be finished by wax polishing, French polishing or varnishing.

*Example 3 red cedar.*

75 The surface of the wood is treated with a solution composed of 1 oz. of ferrous sulphate plus  $\frac{1}{4}$  oz. of potassium bichromate dissolved together in one gallon of water applied as before. When the moisture has evaporated the result will be a warm nut-brown color, 80 which may be finished by wax polishing, French polishing or varnishing.

## I claim:—

1. A process for decoratively coloring the surface of wood, consisting in treating the surface of the wood with a metallic sulphate and a developing reagent.
2. A process for decoratively coloring the surface of wood, consisting in treating the surface of the wood with ferrous sulphate 90 and a developing reagent.
3. A process for decoratively coloring the surface of wood, consisting in treating the surface of the wood with a metallic sulphate and a chromate.
4. A process for decoratively coloring the surface of wood, consisting in treating the surface of the wood with a metallic sulphate and potassium bichromate.
5. A process for decoratively coloring the 100 surface of wood, consisting in first treating the surface of the wood with a metallic sulphate and subsequently with a developing reagent and ammonia.
6. A process for decoratively coloring the 105 surface of wood, consisting in first treating the surface of the wood with a solution including a metallic sulphate, evaporating the moisture from the treated surface, and then treating the surface with a solution including a chromate mixed with liquid ammonia.
7. A process for decoratively coloring the 110

surface of wood, consisting in first treating the surface of the wood with a solution including ferrous sulphate, evaporating the moisture from the treated surface, and then 5 treating the surface with a solution including a chromate mixed with liquid ammonia.

8. A process for decoratively coloring the surface of Oregon pine or wood of like character, consisting in first treating the surface 10 of the wood with a solution including a metallic sulphate, evaporating the moisture from the treated surface, and then treating

the surface with a solution including a chromate mixed with liquid ammonia.

9. A process for decoratively coloring the 15 surface of Oregon pine or wood of like character, consisting in first applying evenly to the surface of the wood a solution including ferrous sulphate, evaporating the moisture from the treated surface, and then treating 20 the surface with a solution including potassium bichromate mixed with liquid ammonia.

MALCOLM SPARKES.